

Feb. 13, 1945.

W. A. HAMILTON

2,369,393

HEAVY MEDIA FINE ORE CONCENTRATION

Filed Oct. 29, 1942



INVENTOR

WALTER A. HAMILTON,

BY  
Robert James Kesten  
ATTORNEY

## UNITED STATES PATENT OFFICE

2,369,393

## HEAVY-MEDIA FINE ORE CONCENTRATION

Walter Arlee Hamilton, Stamford, Conn., assignor to American Cyanamid Company, New York, N. Y., a corporation of Maine

Application October 29, 1942, Serial No. 463,744

2 Claims. (Cl. 209—173)

This invention relates to an improved method of concentration of ores.

Various processes of concentrating ores have been developed using specific gravity methods for separation. Notable success has been obtained by the process which used heavy media produced by the suspension of solids of high specific gravity in water for the separating process. These methods of beneficiation depending on sink and float procedures have been of great importance in the treatment of many ores as the process is extremely cheap and the metallurgical efficiency is much higher than ordinary hydraulic methods. However, there are very definite limitations to the type of ore which is amenable to such separation processes as they do not separate efficiently below a certain minimum size. With many ores either the mining operation itself or subsequent crushing required for liberation of values reduces part or all of the ore to a much finer size than can be practically handled in sink and float processes using heavy media. This is notably true in the beneficiation of various low-grade iron ores.

The economics of iron ore beneficiation is strongly influenced by the fact that the final product commands a low unit price, and hence costs of beneficiation must be kept very low in order to render the process commercially useful. For the most part iron ore crudes requiring beneficiation are concentrated to a moderate degree in comparison with other base metal concentrations. Therefore, processes in which separation is not extremely sharp can be used with iron ores and similar ores where an extreme purity of product is not necessary. It is with these types of ores that the present invention is concerned and it may be considered as a modification or improvement of known procedures. In the further detailed discussion reference will be made primarily to iron ores although the present invention is not limited to such ores and is applicable to any other ores, such as for example manganese ores, where a similar problem arises.

Some of the advantages of the sink and float procedure in heavy media have been extended to the treatment of unsized material, or rather to material which is relatively free from large amounts of fine low density material, using a modified device which is neither a pure sink and float procedure nor an ordinary hindered settling classifier. Such a device and method is described and claimed in the application of Lewis J. Erck, Serial No. 395,809, filed May 29, 1941. According to this procedure an apparatus of the classifier type such as for example an apparatus resembling in its gross structure an Akins classifier is modified and operated by maintaining a high bed of dense suspended solids with only a relatively shallow stream of supernatant water. The density of this deep pool of solids is not sufficiently high to permit a true sink and float separation. That is to say, the true density is below that of light gangue

material. The pool of solids is maintained to a point only a little below the overflow weir of the classifier and the solids pool is worked mechanically by modifications of the Akins screw. The combined mechanical working and up-flow of water results in bringing coarse low density material to the surface and as the amount of water is in general larger than in many classifier operations, a considerable shallow stream of water runs over the surface of the pool and over the overflow weir. This stream carries with it the coarse low density particles which have been worked to the surface of the solids pool and also takes with it a considerable amount of fine high density material. In considering the high density material the action is primarily one of classification because the overflow takes substantially only fine high density material. From the standpoint of the low density material the operation is one depending primarily on specific gravity and mechanical working for its operation. Therefore, this second stage in the process of the Erck application is not an ordinary classification but a concentration. However, the device operates by reason of the upward flow of water to overflow a mixture of relatively coarse light gangue and fine high density material, the underflow being a mixture of coarse and fine high density material. This improved process and device has achieved considerable success in the treatment of unsized fine iron ores and such a device is included in one of the combined steps in the process of the present invention.

Erck describes the use of his concentrator in a number of methods of treatment, some of these procedures being described in the Erck applications, Serial No. 430,342, filed February 11, 1942, and Serial No. 436,419, filed March 27, 1942, and also in an application of Grover J. Holt, Serial No. 437,464, filed April 3, 1942. Essentially these procedures are applicable to iron ores or similar ores where there is present a large amount of fine low density material. The procedures may be briefly summarized as follows:

The unsized iron ore carrying relatively large amounts of finely divided siliceous gangue associated with coarse quartz and both coarse and fine iron ore is subjected to an ordinary free-settling classification which produces an overflow of fine gangue associated with a small amount of very fine iron ore, while the underflow consists of coarse quartz particles and coarse and medium fine iron ore particles. The classification operation may be effected in any suitable classifiers, but in large scale commercial operation on the Minnesota iron ores an ordinary Akins spiral type classifier is normally employed. The underflow or rake product is then fed to an Erck concentrator operating as described above. This concentrator produces two products, an underflow which contains practically all of the coarse iron ore associated with a portion of the medium

fine ore, and an overflow containing substantially all of the coarse light quartz particles associated with the portion of the fine iron particles. This overflow is then subjected to a treatment which removes coarse quartz particles. In commercial practice it is usual to employ a screening procedure, the screen oversize being sent to waste, but if desired, with certain ores where the coarse gangue contains values liberatable at a finer grind, the oversize may be ground to a uniform fine size preliminary to a further treatment. In either event the fine iron ore in the screen undersize is recirculated to the first or primary classifier. Thus it will be seen that when screening is used silica is discharged from the system at two points, both from the oversize of the separating screen and from the overflow of the primary classifier. Where grinding is employed all of the silica is discharged as fine material in the primary classifier overflow.

The procedure of the Erck and Holt applications is used in a large commercial plant on the iron ores of the Mesabi Ranges in Minnesota and is well suited for the treatment of these ores. However, when applied to a different type of iron ore, such as for example ores mined in Alabama, Colorado and the like, the process is not as efficient. These ores are characterized by a relatively lower content of very fine silica, but they are characterized by a relatively high iron content in very fine sizes. If, therefore, the procedures of the Erck and Holt patents are attempted on such ores serious losses in fine iron ore result. According to the present invention the disadvantage of the Erck and Holt processes on ore containing relatively small amounts of low density material and large amounts of fine high density material are overcome and, at the same time in many cases, a much simpler procedure is effected with a notable increase in output per unit of equipment, all important advantages in the treatment of a relatively low valued material. Essentially the present invention shares with the Erck and Holt procedures the combination of a primary classifier and an Erck concentrator, but both overflows of the concentrator and classifier are screened and concentrated and tailings are obtained from both overflows. Recirculation of the undersize from the concentrator overflow is normally not necessary, but if employed at all constitutes only a minor amount of recirculation. There is thus obtained a high degree of recovery of high density values without losses of fine high density material and particularly in some modifications with a greater increase in

through-put due to the fact that little or no material is recirculated, the high recirculating load which is characteristic of the Erck and Holt processes being avoided.

Essentially the present invention, may therefore, be considered as an improvement on the Erck and Holt processes which, however, is applicable to a different class of ore. The two processes have their own place in the economics of iron ore beneficiation, but where the nature of the ore permits, the lowered cost and improved efficiency of the process of the present invention represents a real economic advantage.

The invention will be described in greater detail in conjunction with the drawing in which the figure is a diagrammatic flow sheet for two typical ores.

The flow sheet was based on procedures employed in the beneficiation of two typical iron ores of the Alabama region, being characterized by a relatively large amount of iron values in fine fractions and a comparatively small amount of the silica in the fine fractions, were subjected to the procedure of the present invention, that is to say, the feed was first sent through a primary classifier, which may for example be an ordinary Akins classifier operated to have a heavy overflow as compared to the primary classifiers used in the Erck and Holt processes, followed by treatment of the underflow or rake product in an Erck concentrator, operated as described in the Erck application, Ser. No. 395,809, referred to above. The overflow of the primary classifier was sized on a 35 mesh screen, the oversize representing a barren tailing and the undersize being marketable concentrate. The concentrator overflow was likewise subjected to screening, but preferably on a somewhat coarser screen such as a 28 mesh screen, the oversize rejected, and the undersize mixed with the rake product of the concentrator and the undersize from the 35 mesh screen as finished product.

Metallurgical results appear in the following Tables 1 and 2. In explanation of these results, fraction 1 represents the rake discharge of the concentrator, fraction 2 the overflow of the concentrator, and fraction 3 the overflow of the primary classifier. In the portion of the table under "Recapitulation" the metallurgical results are given on the total marketable concentrate and the total tailing. For convenience the figures are also given on the drawing in Fig. 1. The top line in each case refers to test one and the bottom line to test two.

TABLE I  
Fine ore concentration Test No. 1

| Product               | Percent weight | Assays     |             |                |                          |                                        | Percent distribution |        |        |                  |                                |
|-----------------------|----------------|------------|-------------|----------------|--------------------------|----------------------------------------|----------------------|--------|--------|------------------|--------------------------------|
|                       |                | Percent Fe | Percent CaO | Percent insol. | Percent SiO <sub>2</sub> | Percent Al <sub>2</sub> O <sub>3</sub> | Fe                   | CaO    | Insol. | SiO <sub>2</sub> | Al <sub>2</sub> O <sub>3</sub> |
| Feed.....             | 100.00         | 33.40      | 13.94       | 20.63          | 18.47                    | 3.46                                   | 100.00               | 100.00 | 100.00 | 100.00           | 100.00                         |
| Fraction 1.....       | 24.19          | 35.81      | 13.01       | 16.62          | 14.91                    | 3.20                                   | 25.94                | 22.57  | 19.49  | 19.55            | 22.45                          |
| +28 mesh Frac. 2..... | 28.93          | 25.99      | 15.24       | 30.16          | 27.88                    | 3.54                                   | 22.51                | 31.63  | 42.30  | 43.69            | 29.49                          |
| -28 mesh Frac. 2..... | 8.64           | 44.63      | 10.31       | 12.84          | 10.86                    | 2.88                                   | 11.55                | 6.39   | 5.38   | 5.09             | 6.94                           |
| +35 mesh Frac. 3..... | 2.54           | 13.52      | 23.46       | 33.12          | 30.63                    | 2.90                                   | 1.03                 | 4.28   | 4.03   | 4.22             | 2.02                           |
| -35 mesh Frac. 3..... | 35.70          | 36.46      | 13.72       | 16.64          | 14.19                    | 3.52                                   | 38.97                | 35.13  | 28.80  | 27.45            | 39.30                          |

RECAPITULATION

|                          |        |       |       |       |       |      |        |        |        |        |        |
|--------------------------|--------|-------|-------|-------|-------|------|--------|--------|--------|--------|--------|
| Feed.....                | 100.00 | 33.40 | 13.94 | 20.63 | 18.47 | 3.46 | 100.00 | 100.00 | 100.00 | 100.00 | 100.00 |
| Conc. <sup>1</sup> ..... | 68.53  | 37.26 | 13.04 | 16.15 | 14.04 | 3.45 | 76.46  | 64.09  | 53.67  | 52.09  | 68.49  |
| Tail <sup>2</sup> .....  | 31.47  | 24.98 | 15.41 | 30.37 | 28.12 | 3.47 | 23.54  | 35.91  | 46.33  | 47.91  | 31.51  |

<sup>1</sup>Includes all of fraction 1, plus the minus 28 mesh from fraction 2 and the minus 35 mesh from fraction 3.

<sup>2</sup>Includes plus 28 mesh from fraction 2 and plus 35 mesh from fraction 3.

TABLE II  
Fine ore concentration Test No. 2

| Product          | Percent weight | Assays     |             |                |                          |                                        | Percent distribution |        |        |                  |                                |
|------------------|----------------|------------|-------------|----------------|--------------------------|----------------------------------------|----------------------|--------|--------|------------------|--------------------------------|
|                  |                | Percent Fe | Percent CaO | Percent insol. | Percent SiO <sub>2</sub> | Percent Al <sub>2</sub> O <sub>3</sub> | Fe                   | CaO    | Insol. | SiO <sub>2</sub> | Al <sub>2</sub> O <sub>3</sub> |
| Feed             | 100.00         | 35.30      | 10.70       | 24.78          | 23.60                    | 3.03                                   | 100.00               | 100.00 | 100.00 | 100.00           | 100.00                         |
| Fraction 1       | 20.44          | 38.81      | 9.86        | 21.66          | 20.55                    | 3.16                                   | 22.47                | 18.84  | 17.87  | 17.80            | 21.45                          |
| +28 mesh Frac. 2 | 23.65          | 24.93      | 10.77       | 41.24          | 40.12                    | 2.10                                   | 16.71                | 23.81  | 39.37  | 40.21            | 16.50                          |
| -28 mesh Frac. 2 | 11.77          | 43.86      | 8.30        | 16.48          | 14.89                    | 4.00                                   | 14.62                | 9.13   | 7.83   | 7.42             | 15.51                          |
| +35 mesh Frac. 3 | 5.51           | 16.82      | 15.64       | 49.68          | 43.67                    | 1.90                                   | 2.63                 | 8.06   | 9.95   | 10.21            | 3.30                           |
| -35 mesh Frac. 3 | 38.63          | 39.81      | 11.12       | 16.02          | 14.89                    | 3.38                                   | 43.57                | 40.16  | 24.98  | 24.36            | 43.24                          |

## RECAPITULATION

|                   |        |       |       |       |       |      |        |        |        |        |        |
|-------------------|--------|-------|-------|-------|-------|------|--------|--------|--------|--------|--------|
| Feed              | 100.00 | 35.30 | 10.70 | 24.78 | 23.60 | 3.03 | 100.00 | 100.00 | 100.00 | 100.00 | 100.00 |
| Cone <sup>1</sup> | 70.84  | 40.20 | 10.29 | 17.72 | 16.52 | 3.43 | 80.66  | 68.13  | 50.68  | 49.58  | 80.20  |
| Tail <sup>2</sup> | 29.16  | 23.40 | 11.69 | 41.89 | 40.80 | 2.06 | 19.34  | 31.87  | 49.32  | 50.42  | 19.80  |

<sup>1</sup> Includes all of fraction 1 plus the minus 28-mesh portion of fraction 2 and the minus 35-mesh portion of fraction 3.

<sup>2</sup> Includes all of plus 28 mesh and all of plus 35-mesh portions of fractions 2 and 3 respectively.

It will be noted that in Test 1, 75% of the iron content of the feed is recovered as a marketable concentrate having less than 17% of silica. It is important to note that more than half of the iron recovered is present in the overflow of the primary classifier and would be lost if the ore were subjected to the Erck and Holt processes.

In the case of the second test over 80% of the iron is recovered in a concentrate having less than 17% of silica. In this case an even larger proportion of the recovered iron is found in the primary classifier overflow.

Where there is a considerable amount of barren gangue of sizes intermediate between 28 and 35 mesh the undersize from the 28 mesh screen may be recirculated to the primary classifier which results in the elimination of barren gangue in this size range with some losses of metal values.

The invention has been described in greater detail in conjunction with iron ores for which the present invention is particularly suited. It should be understood, however, that the invention is not limited to the treatment of iron ores and on the contrary is applicable to any ore where there is a large proportion of values present in fine sizes and there is a relatively negligible amount of fine low-density material. As the process in counter distinction to flotation processes does not depend on the constitution of the ore it is applicable to any ores which have the above type of distribution of heavy density and low density materials.

In the treatment of iron ores, manganese ores and most others the valuable product is that of high density. The process, however, is not limited to such ores and on the contrary is applicable to ores such as coal in which the valuable product is that of low density.

The largest field of practical utility lies in the treatment of ores. However, the process is in fact not concerned with the past history of the mixtures of products treated and is applicable to mixtures artificially produced, either by partial beneficiation of natural ores, such as concentrates of various kinds, mixtures obtained by artificial production, and the like. The present invention is also not limited to the process in which the only concentration is that effected by the means of classification, concentration and sizing. On the contrary any of the products may be subjected to further treatments such as for example froth flotation, tabling and the like. The general applicability of the present invention and the possibility of using it in conjunction with other

ore dressing procedures is an important practical advantage which lends great flexibility to the process and which widens its field of usefulness.

25 The primary classifier has been described as one of the hydraulic type and with most ores, notably with iron ores of the type specifically illustrated, hydraulic classification presents many advantages and is the preferred type of classification. However, it should be understood that this primary classification is not necessarily limited in all cases to the use of hydraulic classifiers. With certain particular ores other types of classification, such as for example air classification 30 and the like, may be employed wherever the particular nature of the ore makes such special classification procedure desirable.

We claim:

1. A method of beneficiating mixtures containing components of higher densities and components of lower densities, in which there is a relatively small amount of finely divided material of lower density and a relatively larger amount of finely divided material of higher density, which 40 comprises subjecting the mixture to hydraulic classification to produce an overflow product containing fine high density material and coarser low density material and an underflow product containing coarse and fine high density material 45 and only coarse low density material, screening the overflow to produce an undersize rich in high density material and poor in low density material and an oversize rich in low density material and poor in high density material, subjecting 50 the underflow to a procedure of combined specific gravity and separation and classification, whereby an overflow is produced containing coarse low density material and fine high density material and an underflow is produced containing coarse 55 high density material and substantially free from major portions of coarse low density material, and subjecting the overflow to screening to produce an undersize rich in high density material and poor in low density material and an oversize rich in low density material and poor in high density material, the screening of the overflow containing coarse low density material being at a coarser mesh size than the screening of the overflow of the primary hydraulic classifier.

60 2. A method of beneficiating iron ore containing iron oxide and siliceous gangue, in which there is a relatively small amount of finely divided siliceous gangue and a relatively larger amount of finely divided iron oxide, which comprises subjecting the mixture to hydraulic clas- 65

sification to produce an overflow product containing fine iron oxide and coarser siliceous gangue and an underflow product containing coarse and fine iron oxide and only coarse siliceous gangue, screening the overflow to produce an undersize rich in iron oxide and poor in siliceous gangue and an oversize rich in siliceous gangue and poor in iron oxide, subjecting the underflow to a procedure of combined specific gravity and separation and classification, whereby an overflow is produced containing coarse siliceous gangue and fine iron oxide and an under-

flow is produced containing coarse iron oxide and substantially free from major portions of coarse siliceous gangue, and subjecting the overflow to screening to produce an undersize rich in iron oxide and poor in siliceous gangue and an oversize rich in siliceous gangue and poor in iron oxide, the screening of the overflow containing coarse low density material being at a coarser mesh size than the screening of the overflow of the primary hydraulic classifier.

WALTER ARLEE HAMILTON.